

# UNITED STATES PATENT OFFICE.

WYMAN H. MEADE AND SVEN H. FRIESTEDT, OF CAMDEN, NEW JERSEY.

## METHOD OF COLORING AND FINISHING THE SURFACE OF GRAIN-LEATHER.

1,376,961.

Specification of Letters Patent.

Patented May 3, 1921.

No Drawing.

Application filed July 24, 1919. Serial No. 313,006.

*To all whom it may concern:*

Be it known that we, WYMAN H. MEADE, a citizen of the United States, and SVEN H. FRIESTEDT, a subject of the King of Sweden, both residing at Camden, county of Camden, and State of New Jersey, have invented certain new and useful Improvements in Methods of Coloring and Finishing the Surface of Grain-Leather, of which the following is a specification.

It has always been difficult to provide an even shade of coloring to the surface of grain leather, especially when light shades of color were desired. Numerous processes have been devised for securing light even shades by coating the leather with a heavy coating of pigment, thereby giving the shades but destroying the natural appearance of the grain of the leather in view of the fact that in order to cover up any variation in shade of the natural leather, heavy coatings of the pigment were applied, said coatings being of sufficient thickness to fill the interstices and recesses on the surface of the leather thereby destroying the natural characteristics of the surface of the leather.

One object of our invention is to color and finish the surface of grain leather in such manner that when extremely light color effects are produced, the color will be even throughout the entire surface irrespective of any variation in color of the natural and at the same time the effect of the natural grain of the leather will not be destroyed. While we have described the main object as the production of light color effects, it will be understood however that our process is equally advantageous for dark effects, since even though the variation in color in the old method of coloring is not as noticeable in dark effects, nevertheless it is noticeable in many instances and by using our process, variation in shade of coloring is eliminated for all shades produced.

The above objects, and other advantageous ends which will be described hereinafter, we attain in the following manner.

Our invention consists primarily of applying an element to the surface of the leather; the element being secured by precipitation, for example, we take any com-

pound which is soluble and precipitate an element therefrom. The element thus precipitated is used as a pigment for applying to the surface of the leather. This precipitate can be applied to the grain-side of the leather in any way as a pigment either dry or mixed with a suitable carrier for covering or coloring the grain of the leather. In view of the extreme fineness of the particles of the pigment produced by the precipitation, the application of this pigment will not destroy the wavy appearance of the leather and any instance where the pigment thus precipitated is metallic, as will be described hereinafter, there is no chance of transparency so that the finished leather will have the color of the precipitated pigment applied thereto.

One way of carrying out our invention is as follows:—

Dissolve 249 parts of copper sulfate ( $\text{CuSO}_4 \cdot 5\text{H}_2\text{O}$ ) in water and add slowly 65 to 70 parts of zinc-dust. Then filter off 75 the precipitated metallic copper, wash free from soluble zinc salt. Then wash it with alcohol and dry at room temperature. When dry it is ready to apply to the leather either in dry form or mixed with some other 80 pigment or carrying agent. One way to do this is as follows:—

Take 50 parts of the element made as above described, mix it with 200 parts of casein solution as carrier. Then apply to 85 the leather and finish the same in any of the well known methods. To produce various effects other well known materials may be added.

Having thus described our invention, 90 what we claim as new and desire to secure by Letters Patent is:—

As a new article of manufacture, leather having a surface coated by metal precipitated from a soluble compound.

In testimony whereof we have signed our names to this specification in the presence of two subscribing witnesses.

WYMAN H. MEADE.  
SVEN H. FRIESTEDT.

Witnesses:

CHAS. E. POTTS,  
ANNA RENTON.